

Feb. 19, 1952

L. PARKER

2,586,250

HEAT EXCHANGER

Filed Sept. 12, 1949

2 SHEETS—SHEET 1

*Fig. 1.*



*Fig. 2.*



*Fig. 5.*



*Fig. 3.*



*Fig. 4.*



INVENTOR.  
**LEON PARKER**  
BY  
*Philip Subkow*  
ATTORNEY.

Feb. 19, 1952

L. PARKER

2,586,250

HEAT EXCHANGER

Filed Sept. 12, 1949

2 SHEETS—SHEET 2

*Fig. 6.*



*Fig. 7.*



*Fig. 8.*



*Fig. 9.*



*Fig. 11.*



INVENTOR.  
LEON PARKER  
BY  
Philip Lubkin

ATTORNEY.

## UNITED STATES PATENT OFFICE

2,586,250

## HEAT EXCHANGER

Leon Parker, Burbank, Calif., assignor to The  
H. I. Thompson Company, Los Angeles, Calif.,  
a corporation of California

Application September 12, 1949, Serial No. 115,242

8 Claims. (Cl. 263—51)

1

This invention relates to regenerative heat exchange apparatus operable at high ambient temperatures and over large ranges of temperatures. It is particularly designed for use with jet or turbo-jet airplane engines wherein the temperatures may range from 900° F. to 1500° F.

In such units it is desired to devise a regenerative heat exchange structure of low pressure drop, high stability against thermal and mechanical shock and corrosion resistance, and of low bulk volume and weight.

I have devised a regenerative heat exchange medium which has the desirable properties specified above. It is formed of silica filaments arranged to present unobstructed longitudinal passageways, preferably by employing textiles, such as woven, knit, corded, braided material or any other interlaced or interwoven silica fibers. The interwoven silica fibers are arranged in a chamber so as to present elongated unobstructed channels through the chamber in the direction of flow of the material, the interwoven silica fibers forming the walls of the channels, which walls may be, if desired, either foraminous or substantially impermeable to the gases passed through the heat exchange apparatus.

Silica has the useful properties for this purpose in that of all solid materials which soften or melt above the temperatures previously referred to, it has a relatively high specific heat and is not corroded or eroded by high temperatures, high velocity combustion gases, or by air at high temperatures moving at high velocity.

While fused quartz, in tubular or massive form, has a low coefficient of expansion and is relatively weak to thermal and mechanical shock, in filamentary form, as yarn, batt, woven, knitted, braided and corded fibers, and, in fact, in any interlaced textile form, the silica fibers have a high degree of stability against thermal shock, and the ratio of exposed surface to total volume of the silica is extremely high. The textile material has a high degree of bulk flexibility, but has little or no rigidity. The textile also may have a high porosity, depending upon the weave, knit or braid pattern employed.

I have found that if this textile is arranged so as to present longitudinal passageways, the textile acting as the separating wall of the passageways, a heat exchange apparatus of very low pressure drop and high efficiency, small volume and high heat capacity results which will be stable to thermal and mechanical shock.

In order to support the fabric to present the aforementioned small pressure drop but to as-

2

sure that it has a high ratio of wall surface to volume of the passageways, I have found it desirable that the passageways be channels of relatively small cross sectional area but of considerable longitudinal dimension in direction of flow so arranged as to introduce little or no obstruction to flow but insure adequate and rapid heat transfer from the gases to the walls. To obtain this effect I have found it desirable to form the heat exchange apparatus of a multiplicity of longitudinally parallel channels the cross sections of which are but a small fraction of their length, but to use a sufficiently large number of these parallel channels so that the free area of the channels is large. Since the walls of the channels are very thin, depending upon the thickness of the yarn and the nature of the weave, the total cross sectional area of the free space may be made the major part of the total cross sectional area and, in fact, the cross sectional area occupied by the textile walls forms but a small percentage of the total cross sectional area. The difficulty in arranging such passageways resides in the inherent lack of rigidity of the fabrics.

I have found it desirable to avoid employing a framework or skeleton to support the textile material when arranged in the manner described above, since it reduces the free area and increases the pressure drop and also adds weight to the heat exchange apparatus.

I have found that I may construct such a siliceous textile so that it has sufficient rigidity to retain its shape and resist deformation due to either thermal or mechanical shock or mechanical deformation without using any framework or structure which will be positioned in the free space. I have accomplished this by using a silica textile formed of interwoven silica filament and metallic wire filaments. The metallic wire forms a skeleton which is much more rigid than the silica textile and will support the silica fibers in any desired conformation. Since the wires are positioned in the textile as a component thereof, they occupy no portion of the free volume. By employing wire having a high tensile strength, rigidity, and corrosion resistance, I may use relatively thin wires and thus reduce the bulk and weight of the non-siliceous portion of the textile.

It has been recently discovered that ordinary glass fibers usually employed in making glass fiber textures may be extracted to remove the glass making oxides, other than silica, and to leave a highly siliceous material in which the silica element may run from 90% to over 99+%

of the oxide element of the extracted material. The extracted material is hydrated and in firing at high temperature the material is dehydrated and shrunk. Reference may be had to the Nordberg Patent No. 2,461,841 and to application Serial No. 669,098, filed May 11, 1946, now Patent No. 2,491,761, by Leon Parker and Alexander Cole, for details of this process.

This procedure results in a large impairment in the tensile strength of the glass fabric. While careful control of the extraction and the washing process will give silica fabrics of relatively high tensile strength, the resultant tensile strength is at best much lower than that of the original glass fiber material.

It is difficult to weave, knit, braid, or cord silica fibers thus produced because of its inherent low strength and therefore it has not been practicable to form the desired composite textile formed of metallic wire and silica fibers for the above use. In my co-pending application, Serial No. 114,998, filed September 10, 1949, I have disclosed procedures whereby this may be accomplished. Instead of weaving or knitting the composite textile using the extracted or extracted and fired silica fibers in thread or yarn form, I first form the textile by weaving or knitting the textile using glass fibers and the other filamentary material to be incorporated in the composite textile. The composite fabric may then be leached to remove from the glass filaments the glass forming oxides other than silica in the usual manner. The composite fiber may then be fired if desired.

The fiber other than glass employed should preferably be immune to chemical or physical attack by the leaching solution in a degree to materially impair its physical or chemical properties.

Glass filaments are leachable either with water alone or by acids, depending upon the nature of the glass. The nature of the glasses and their relation to and method for leaching such glasses are described in the above mentioned Norberg patent and the Parker-Cole application.

Thus, if the glass filament is leachable with water as, for example, the alkali boro-silicate glass having a high boron-oxide to alkali ratio, for example, not less than about 5:1, I may employ almost any other filament in forming the original composite glass cloth, for example, any of the filaments referred to above, since they will not be impaired by the water. In fact, most filamentary material, such as is used for weaving, knitting, braiding, cording or other textile forming process, whether metallic or non-metallic, or organic or inorganic, such as the glass, not leachable by water, may be used, since what is desired is a fiber which will not be attacked by water or attack by water will not be significant in reducing its strength to a relatively low value. I may extract the glass cloth by prolonged attack by water to remove the non-siliceous oxides and thus give a leached composite cloth of higher tensile strength than can be obtained by leaching a textile formed of the leachable glass fibers. When I employ a glass fiber which is leachable with water, I may form a composite fabric formed of water leachable glass and also of glass which is immune to attack by such water. Such glasses are the boro-silicate glasses having 70% or more of  $\text{SiO}_2$ , and if containing less than 70%, those which are substantially free from alkali metal oxides but which contain substantial amounts of second group oxides and alumina or any other type of

glass filaments composed of  $\text{SiO}_2$  and other water insoluble glass forming oxides.

Where the glass fibers are not leachable by water but require an acid leaching agent, such as HCl, as is the case with those glasses the properties of which make them particularly suitable for formation into filaments suitable for textile manufacture and which are now widely used for this purpose, I prefer to use as the added tensile-strength-imparting filament material one which is resistant to attack by the acid.

The acid leachable glass fibers are characterized by being formed from boro-silicate glasses substantially free from alkali and containing substantial amounts of second group oxides and alumina, for example, 56% or less of  $\text{SiO}_2$ , about 22% or less of second group oxides, about 12% or more of  $\text{Al}_2\text{O}_3$ , and about 5% or more of  $\text{B}_2\text{O}_3$ . Soda-lime glasses may also be leached with acid, 20 i. e., those containing about 20% or more of alkali and about 75% or less of  $\text{SiO}_2$  and containing second group oxides.

I have found that for my purposes, because of their adaptability to forming glass filaments and 25 textiles, the acid leachable boro-silicate glasses are to be preferred.

I, therefore incorporate as the added strength-imparting filament one which is resistant to such attack by acid and preferably by acid at the 30 elevated leaching temperatures employed. Such filaments are the acid resistant glass filaments and acid resistant organic synthetic fibers such as polyvinylidene chloride, polyvinyl chloride, and the noncorrosive metallic wires listed below. All 35 of these materials form a natural group in that they can be formed into filaments which can be formed into textiles and resist chemical attack by HCl at elevated temperatures above 100° F. and below 212° F., which temperatures are usually 40 employed in the glass leaching operation.

However, if the textile is to be fired to dehydrate it, I must use as the fiber, other than the leachable glass fiber, a material which will be stable at the elevated firing temperature of about 750° F. and preferably as high as 1600° F. at 45 which the textile is fired. In such circumstances I cannot use the organic fibers, natural or synthetic, since they will be destroyed by firing and glass filaments will lose their strength by devitrification or may actually melt if the higher temperatures are used. In such circumstance I prefer to employ filaments of material which will be stable at the high temperatures used for dehydration and shrinkage of the leached fabrics.

55 I thus prefer to use the metallic filaments. Many metals are available in fine wire form and may be handled on conventional braiding, cording, weaving or knitting machines. These include copper, steel, nickel, chromium, nickel-molybdenum, and many others which will suggest themselves to those skilled in this art. However, if the leaching agent be acid, I must select those which are not corroded by acid, and thus I prefer to employ the acid resistant filaments made of 60 Hastelloy B (whose composition is referred to below), platinum, tantalum, Phosphor bronze, aluminum-bronze, gold, silver, nickel-silver alloy, Everdur, which is a copper, silicon, manganese alloy, copper ranging from 94.9 to 98.2%, silicon 65 1.5 to 4%; manganese 0.25 to 1.1%, and also chromium-copper alloys. The metallic wires which have a melting point at about 1500° F. or higher form a sub-group of the acid resistant metallic wire group referred to above in that they 70 are not only acid resistant, as described above,

but will be stable when the composite textile is fired or used at temperatures of 1500° F.

I, therefore, distinguish the filaments employed in my composite textile formed of such interlaced filaments as leachable glass filaments and non-leachable reinforcing filaments, meaning that under the conditions of leaching wherein I extract the non-siliceous glass oxides of the leachable glass to produce silica fibers containing non-siliceous oxides in the ratio of 9:1 or more of silica to non-metallic oxides, the non-leachable fibers will not be attacked in any substantial manner during such leaching, and I refer to the latter as a reinforcing filament in that the properties of the composite fabric, such as tensile strength and abrasion resistance, are enhanced by their presence in the reinforced fabric above that formed of the siliceous material alone.

The properties of the resultant leached fibers thus formed into a composite textile material include resistance to acid or water attack. The fired silica fibers are not attacked by alkali. The fusion and softening points are high above 1600° F., depending upon the amount of leaching and the melting and softening points may be as high as 2000° F. or more.

The dried silica fibers (dried below about 385° F.) and unfired silica fibers have desiccant properties. The fibers are soft, and before and after firing are soft and silky and resemble silk even more than do the original glass fibers.

I prefer to employ the wires which belong to this sub-group since, as will be indicated below, I prefer to use the acid leachable glass filaments.

On firing the glass filament woven into a composite fabric, the silica shrinks while the metallic wires do not. This shrinkage causes a crinkling of the wires so as to cause them to protrude from the surface of the fabric in the form of hooks or loops. Superposed fabric is thus interlaced and locked in position.

I have thus developed a heat exchange apparatus composed of a plurality of channels separated by walls formed of a composite textile material, which composite textile material is composed of interlaced silica and metallic wire filaments.

This invention will be further described in connection with the drawings, in which

Fig. 1 is a showing somewhat schematic of a vertical section of a regenerative heat exchanger such as forms the subject matter of this invention;

Fig. 2 is a plan view somewhat schematic of a tubular woven fabric which may be used in the exchanger of Fig. 1;

Fig. 3 is a section taken on line 3—3 of Fig. 2; of an extracted tubular woven fabric before firing;

Fig. 4 is a section of Fig. 3 of the tubular material after firing;

Fig. 5 is a perspective, somewhat schematic showing, of the stacked tubing showing the interlocking thereof;

Fig. 6 is a somewhat schematic showing of a knitted tape which may be used in another form of the invention;

Fig. 7 is a section taken on line 7—7 of Fig. 6, showing the section after the fabric is leached before it is fired;

Fig. 8 is a section similar to Fig. 7, showing the leached and fired fabric;

Fig. 9 shows the fabric of Fig. 6 corrugated;

Fig. 10 shows one method of stacking such corrugated fabric to give the longitudinal passageways shown in Fig. 1;

Fig. 11 is a perspective of the fabric of Fig. 9 corrugated for stacking as in Fig. 10.

The heat exchange unit of Fig. 1 is composed of a box 1 of any desired cross section, whether circular, square or otherwise, having an inlet 2 and outlet 3 for gases. The heat exchange contact material, shown schematically at 4, may be positioned between two retaining screens 5 and 6. The heat exchange material may be of the form shown in Figs. 4 and 5, that is, of tubular woven character. Fig. 6 shows schematically the nature of the weave composed of the metallic filament 7 and leachable glass fiber filaments 8. These are woven in tubular fashion on a standard tubular braiding machine and results in a tubular fabric having pore spaces in the walls between the fabric filaments and a composite wall composed of the metallic filaments 9 and the glass filaments 8. The metallic fibers, even if the same number of threads of metallic fibers and glass fibers is employed, are such that the exposed area is a major part of the glass.

As examples of this type of reinforced silica fiber cloth, the following may be taken as illustrative, but not as a limitation of the invention.

A tubular braid may be formed using .007" diameter dead soft Hastelloy B wire having the following composition: C, 0.12%; Mo, 26-30%; Fe, 4-7%, and Ni on balance to make 100%.

This is braided with glass fiber yarn .01" in diameter (made of glass fibers each less than .001" in diameter) having the following composition:

The glass fiber had 2.09% organic matter, being the lubricant employed in the weaving. The material was burned off and the loss in weight (2.09%) is here reported as lubricant. The residual 97.91% had the following composition on a lubricant free basis:

|                                | Per cent |
|--------------------------------|----------|
| SiO <sub>2</sub>               | 53.95    |
| Al <sub>2</sub> O <sub>3</sub> | 16.14    |
| Fe <sub>2</sub> O <sub>3</sub> | .56      |
| CaO                            | 15.96    |
| MgO                            | 4.10     |
| B <sub>2</sub> O <sub>3</sub>  | 8.20     |
| Na <sub>2</sub> O              | .88      |
|                                | 99.79    |

The braiding machine, for example, may have 24 carriers, using 12 carriers of wire and 12 carriers of glass fibers with two ends per carrier and 14 picks per inch. Figs. 6, 7, 2, and 3 illustrate the nature of the resulting tubular woven material. The braiding may be leached by any strong acid, preferably one whose salts of the non-siliceous metal oxides are soluble in water; for example, HNO<sub>3</sub>, HCl, chloroacetic acid. Thus, for example, the braiding can be leached with 12% hydrochloric acid solution for 2 hours at 170° F., then washed in water until chloride free, when the water has a pH of about 7-8. The wire is not attacked by the acid and no discoloration of the glass cloth results. The leaching operation is conducted until the silica ratio to the remaining non-siliceous oxides is about 9:1 or more, preferably until the total silica content based on the fired dehydrated silica filament is 95 to about 99+%. The leached fibers have the conformation and arrangement of the original fibers of the composite textiles, as is illustrated in Figs. 2, 3, 6 and 7.

The resultant sleeving has the characteristic of look and feel as sleeving produced when only 75 glass cloth is leached. The revealed wires appear

uniformly spaced over the surface of the sleeving. The sleeving is many times stronger in tension as compared to sleeving similarly formed of fine glass fibers containing no wire. The wires impart a rigidity to the sleeving not present when no wire is used and can be flexed to any desired shape and when so flexed will hold its shape. The sleeving is then fired at an elevated temperature to dehydrate the silica, for example, at 1500° F. for 20 minutes. The silica shrinks and causes a crinkling of the wires. As a result the wires where they are revealed at the surface appear to be crimped, thus giving a series of hook-like projections 9a. These tubes can then be stacked between the screens 5 and 6 to give a plurality of longitudinal passageways with porous walls, through and around the stacked tubes. The hook-like projections 9a interlock, holding the ends in place relative to each other, resulting in a compact stable structure. The natural bulk flexibility of the fabric tubes makes them resistant to mechanical and thermal shock. The weight of the tubular material per inch was  $4.3 \times 10^{-4}$  pounds and about 2.9 pounds per square feet of cross-sectional area one inch thick in the heat exchanger 1.

Instead of the fibers of .01" in diameter used in the previous example, a glass fiber of .0065" in diameter may be used which would result in a leached and fired sleeving of .1057" internal diameter. All of these sleeveings will have the necessary rigidity to maintain their shape and will be interlocked in the manner described above by the use of any framing other than the structure of the sleeve itself.

Instead of using sleeving, I may use tape which may be corrugated in the form shown in Figs. 9, 10, and 11. For example, these figures illustrate the use of wires of different diameters to be interwoven with the tape. Thus, in Figs. 9, 10, and 11 the wire of .007" diameter, of the type previously described illustrating the formation of the tubes, was employed as the warp and a wire of .003" diameter was employed as fill, shown at 10, spacing the warp more closely than the fill. The glass fiber of .0065" diameter was interknit on a standard tape knitting machine. The tape was then leached in the manner as described for the tube and fired in the same way. The finished tape was  $\frac{3}{4}$ " wide, and had a thickness of .029". The tape was woven to  $1\frac{1}{8}$ " wide, and after leaching and firing it finished as  $\frac{15}{16}$ " wide and .019" thick and a weight of .009 pound per foot. This tape was corrugated  $\frac{1}{4}$ " overall height and  $\frac{1}{8}$ " between corrugations, as illustrated in Fig. 11, the tapes being stacked side-by-side across the width of the heat exchanger to give tubular passageways 11. The interlocking of the protruding metallic hooks positions these several layers of corrugated tape which tape holds its form after corrugation and is retained snugly in the heat exchanger shell between the screens 4 and 5.

While I have described a particular embodiment of my invention for the purpose of illustration, it should be understood that various modifications and adaptations thereof may be made within the spirit of the invention as set forth in the appended claims.

I claim:

1. A heat exchange unit, comprising a housing, a fluid inlet, a fluid outlet from said housing, a plurality of elongated fluid passageways through said housing, the said passageways having walls

comprising textile material formed of interlaced silica filaments.

5 2. A heat exchange unit, comprising a housing, a fluid inlet, a fluid outlet from said housing, a plurality of elongated fluid passageways through said housing, the said passageways having walls comprising textile material formed of interlaced silica filaments containing non-siliceous metallic oxides, the ratio of silica to non-siliceous metallic oxides being at least 9:1 said silica filaments having a fusion point in excess of 1600° F.

10 3. A heat exchange unit, comprising a housing, a fluid inlet, a fluid outlet from said housing, a plurality of elongated fluid passageways through said housing, the said passageways having walls comprising textile material formed of interlaced metallic filaments and silica filaments.

15 4. A heat exchange unit, comprising a housing, a fluid inlet, a fluid outlet from said housing, a plurality of elongated fluid passageways through said housing, the said passageways having walls comprising textile materials formed of interlaced metallic filaments and silica filaments, said silica filaments containing non-siliceous metallic oxides, the ratio of silica to non-siliceous metallic oxides being at least 9:1 said silica filaments having a fusion point in excess of 1600° F.

20 5. A heat exchange unit, comprising a housing, a fluid inlet, a fluid outlet from said housing, a plurality of elongated fluid passageways through said housing, the said passageways having walls comprising tubular textile material formed of interlaced silica filaments.

25 6. A heat exchange unit, comprising a housing, a fluid inlet, a fluid outlet from said housing, a plurality of elongated fluid passageways through said housing, the said passageways having walls comprising tubular textile material formed of interlaced silica filaments containing non-siliceous metallic oxides, the ratio of silica to non-siliceous metallic oxides being at least 9:1 said silica filaments having a fusion point in excess of 1600° F.

30 7. A heat exchange unit, comprising a housing, a fluid inlet, a fluid outlet from said housing, a plurality of elongated fluid passageways through said housing, the said passageways having walls comprising tubular textile material formed of interlaced metallic filaments and silica filaments.

35 8. A heat exchange unit, comprising a housing, a fluid inlet, a fluid outlet from said housing, a plurality of elongated fluid passageways through said housing, the said passageways having walls comprising tubular textile material formed of interlaced metallic filaments and silica filaments containing non-siliceous metallic oxides, the ratio of silica to non-siliceous metallic oxides being at least 9:1 said silica filaments having a fusion point in excess of 1600° F.

40 LEON PARKER.

#### 60 REFERENCES CITED

The following references are of record in the file of this patent:

#### 65 UNITED STATES PATENTS

| Number    | Name     | Date           |
|-----------|----------|----------------|
| 1,418,234 | Cleary   | May 30, 1922   |
| 1,745,113 | Odell    | Jan. 28, 1930  |
| 1,879,056 | Brassert | Sept. 27, 1932 |
| 2,381,218 | Jacob    | Aug. 9, 1945   |
| 2,385,577 | Jacob    | Sept. 25, 1945 |